

# United States Patent

[19]

Versorese

[11] 3,854,948

[45] Dec. 17, 1974

[54] **NEW DEVELOPMENT COMPOSITION FOR  
RADIOGRAPHIC FILM**

[75] Inventor: **Walfredo Versorese**, Savona, Italy

[73] Assignee: **Minnesota Mining and  
Manufacturing Company**, St. Paul,  
Minn.

[22] Filed: **May 15, 1972**

[21] Appl. No.: **253,428**

[30] **Foreign Application Priority Data**

May 15, 1971 Italy ..... 50368/71

[52] **U.S. Cl.** ..... **96/66 R**, 96/66.3, 96/66.4,  
250/477

[51] **Int. Cl.** ..... **G03c 5/30**

[58] **Field of Search** ..... 96/66 HD, 61 M, 48 PD,  
96/29, 66; 250/320, 323, 477

[56] **References Cited**

UNITED STATES PATENTS

2,751,300 6/1956 James et al. ..... 96/29 R  
3,186,842 6/1965 DeHaes et al. ..... 96/66 R

|           |         |                     |          |
|-----------|---------|---------------------|----------|
| 3,312,550 | 4/1967  | Stewart et al. .... | 96/66 HD |
| 3,345,174 | 10/1967 | Dotson et al. ....  | 96/50 R  |
| 3,431,108 | 3/1969  | Willemens ....      | 96/29 R  |
| 3,567,443 | 3/1971  | DeHaes ....         | 96/29 R  |
| 3,615,512 | 10/1971 | Ducrocq ....        | 96/29 R  |
| 3,702,246 | 11/1972 | Ohyama ....         | 96/29 R  |

OTHER PUBLICATIONS

Mason, Photographic Chemistry, pp. 149-151.

*Primary Examiner*—Norman G. Torchin

*Assistant Examiner*—M. F. Kelley

*Attorney, Agent, or Firm*—Alexander, Sell, Steldt & DeLahunt

[57] **ABSTRACT**

A photographic developer solution for manual processing of photographic [radiographic] film said solution comprising from about 10 to 30 grams per liter of hydroquinone, from about 0.3 to 0.9 grams per liter of phenidone, and further comprising a source of thiosulfate ion in an amount equivalent to from about 0.1 to 1.0 grams per liter of sodium thiosulfate.

**10 Claims, No Drawings**

## NEW DEVELOPMENT COMPOSITION FOR RADIOGRAPHIC FILM

The present invention relates to liquid photographic developer compositions and particularly to such compositions useful for developing radiographic films of the type designed for automatic machine processing.

Certain presently-available photographic films are designed for rapid (e.g., 90 seconds or less) machine processing. Such processing normally employs temperatures in the range of 35°C, and utilizes specially-formulated radiographic film characterized by containing a comparatively small quantity of silver (such as 9.0 grams per square meter) and by a comparatively high silver/gelatin ratio, which may often be higher than 1.2. Reduced quantities of gelatin permit rapid drying of radiographic film. Machine processing (e.g., machine development) involves passage of a film at relatively high temperatures between various rollers which knead and impregnate the film with developer liquid, permitting the film to develop acceptable maximum densities and contrasts, even when considering the relatively low quantities of silver in such machine-processable films.

Until now, however, machine-processable films (e.g., those characterized as above) have not provided completely satisfactory results when manually developed in the same solutions used for machine development. The reasons for this phenomenon are believed to include the lower temperatures ordinarily used for manual development and the lack of thorough contact between liquid developer and radiographic emulsion which is available through machine processing. Accordingly, radiographic film producers have ordinarily prepared two types of radiographic films, one suitable for machine development and the other suitable for manual development.

It is an object of the present invention to provide a liquid photographic developer for manual development of machine-processable radiographic film.

It is another object of the invention to provide a method for manual development of machine-processable photographic film.

Liquid developers normally employed in machine processing include hydroquinone and phenidone as developing agents, an antioxidant such as an alkali sulfite (e.g., sodium sulfite), a development inhibitor such as an alkali bromide, an alkalinizing agent for raising pH, such alkali metal and ammonium hydroxides or sodium carbonate, etc., a pH controlling agent such as an alkali metal metaborate or tetraborate, and an organic fog-inhibiting agent such as benzotriazole, 5-methylbenzotriazole, 6-nitro-benzimidazole and 1-phenyl-5-mercaptopotetrazole, etc. Such compositions ordinarily also include an anticalcium substance such as an alkali polyphosphate, or alkali salts of the ethylenediaminetetraacetic acid type. Such developers can be, if desired, marketed as concentrated liquids to be diluted prior to use, for example, in a one-fourth or one-fifth ratio. For ease of packaging, liquid developer components can be divided into several, separately packaged portions. For example, in one instance it may be desirable to divide the liquid developer into two concentrated portions, one acidic in nature and the other basic in nature. Such portions, when mixed and diluted, will provide a developing solution ready for use ("working solution"). The portion which is basic in nature will

have a pH normally higher than the intended working solution, and may tolerate a high concentration of hydroquinone if desired. Phenidone can be included in the alkaline portion, in the acid portion, or can be divided between the two portions.

Various other liquid developer components as mentioned above may be distributed between the concentrated portions as desired. For example, the basic portion may include the pH control agent and antioxidant, whereas the acid portion may include the development inhibitor and fog inhibitor. It will be understood that the developer of the invention, and the various concentrated portions as mentioned above, are aqueous in nature.

15 The hydroquinone and phenidone components of the above-described liquid photographic developers are ordinarily used within concentration limits known to the art. Preferably, hydroquinone is employed in amounts ranging from about 10 to about 30 grams per liter, and phenidone is employed in amounts ranging from about 0.3 to about 0.9 grams per liter. The pH of such liquid developers is ordinarily in the range of from about 10 to about 11 (preferably 10.2 to 10.5), and may be regulated by use of an alkalizing agent.

20 According to the present invention, it has been found that the hydroquinone/phenidone liquid developer compositions of the type hereinabove described may be modified so as to permit excellent results to be obtained in manual development of machine-processable radiographic films. The modification comprises incorporating into such liquid developers a source of thiosulfate ions in an amount equivalent, in thiosulfate ions, to from about 0.1 to about 1.0 grams per liter of sodium thiosulfate.

25 30 35 Thus, briefly, the present invention relates to a liquid photographic developer having a pH of from about 10 to about 11 (preferably from about 10.2 to about 10.5) and comprising from about 10 to about 30 grams per liter of hydroquinone and about 0.3 to about 0.9 grams per liter of phenidone, the developer being characterized by including a source of thiosulfate ions in an amount equivalent, in thiosulfate ions, to from about 0.1 to about 1.0 grams per liter of sodium thiosulfate.

40 45 50 55 60 65 In an effort to improve the manual development characteristics of machine-processable radiographic films developed with known liquid photographic developers of the hydroquinone/phenidone type, various substances of the thiourea, sodium thiosulfate, and potassium sulfocyanate type have been added to the developer. These are substances which conform soluble complexes with silver ions or can originate salts with solubility products higher than the solubility product of the silver halide present in the radiographic emulsion, or can free ions which will complex silver ions as water-soluble complex salts. Such substances, however, have not been found to yield beneficial results. Surprisingly, it has been found according to the present invention that the addition of a source of thiosulfate, such as sodium or ammonium thiosulfate, in an amount equivalent, in thiosulfate ion, to sodium thiosulfate in an amount of from 0.1 to 1 gram per liter of working solution, yields unusually good results when the resulting working solution is employed for manual development of a machine-processable radiographic film. This is a unique result in view of the fact that the resulting solutions do not show a beneficial improvement when em-

ployed in machine processing of machine-processable radiographic films.

The liquid photographic developers of the present invention may, of course, contain the various developer additives as previously exemplified, and may be packaged as concentrates as exemplified above. The optimum amount of thiosulfate which is added to hydroquinone/phenidone liquid developers to form the developers of the invention may vary according to the type of developer which is used and the type of radiographic material which is developed, and this amount can be easily determined by the skilled artisan. It has been found, however, that the amount of the source of thiosulfate ions can vary only within certain predetermined limits; these limits corresponding to thiosulfate ions in an amount equivalent to from about 0.1 to about 1.0 grams of sodium thiosulfate per liter of working solution.

The invention may be more easily understood by reference to the following illustrative, non-limiting examples.

#### EXAMPLE 1

A medical radiographic film, suitable for rapid machine processing (Minnesota Mining and Manufacturing Company Medical X-Ray film type R) comprising a silver bromoiodide emulsion with about 9 g of silver per square meter and a silver/gelatin ratio of 1.80 was radiographically exposed and then divided into three portions.

The first portion was processed by machine using a processing cycle of 90 seconds at 33°C (a Kodak X-OMAT M6-RP X-Ray Processor) comprising as development solution the Kodak RP Medical X-OMAT Developer-Replenisher type MX 810. The second portion was processed in a manual processing cycle of 3.5 at 20°C using a development bath obtained by dilution of a concentrated liquid development composition consisting of two parts, A and B with the following relative composition:

#### PART A

|                                                                                        |          |
|----------------------------------------------------------------------------------------|----------|
| Water at 20°C                                                                          | 400 cc   |
| Hydroquinone                                                                           | 84.00 g  |
| Phenidone                                                                              | 2.80 g   |
| Sodium Tetaborate                                                                      | 32.00 g  |
| Sodium Metabisulfite                                                                   | 120.00 g |
| Potassium hydroxide (35% p/w solution, D/20°C = 1.341)                                 | 394.70 g |
| Trisodium salt of the hydroxyethyl-ethylene-diamine-triaceitic acid (41% p/w solution) | 18.40 g  |
| Water at 20°C                                                                          | 1000 cc  |

#### PART B

|                                     |          |
|-------------------------------------|----------|
| Water at 20°C                       | 350 cc   |
| Acetic acid 80% p/w (D/20°C = 1.07) | 590.90 g |
| 1-phenyl-5-mercapto-tetrazole       | 1.21 g   |
| Potassium bromide                   | 101.00 g |
| Water to                            | 1000 cc  |

The "working" development solution (solution C) was obtained by dilution of 250 cc of part A with 750 cc of common water and adding 20 cc of part B in order to obtain a final pH of 10.35.

The third part of the film was processed in a manual processing cycle of 3.5, wholly equivalent to the pre-

ceding cycle, except that the processing bath included sodium thiosulfate present in part A of the concentrated liquid development composition in amount of 2.02 g.

The results obtained are given in the following table.

TABLE 1

|        | Fog  | Relative Sensitivity | Average Contrast | Maximum Density |
|--------|------|----------------------|------------------|-----------------|
| Part 1 | 0.22 | 7.8                  | 2.64             | 3.39            |
| Part 2 | 0.20 | 6.5                  | 2.30             | 2.50            |
| Part 3 | 0.20 | 7.0                  | 2.60             | 3.22            |

#### EXAMPLE 2

Samples of various radiographic films (Radio Medica Type N, Radio Industriale Gamma and Radio Industriale Lambda, all of 3M Company) having emulsions with concentrations of silver per square meter of 9, 10, 9.7, and 24 g, respectively, and having respective silver/gelatin ratios of 1.80, 0.63, 0.4, and 1.00, were exposed radiographically, and then cut into several strips. Each of these strips was processed in a manual processing cycle of 3.5 at 20°C employing various types of development baths, wholly analogous to the solution C of Example 1. Each development bath was either devoid of other additives or included sodium thiosulfate, sulfocyanate and thiourea in the amounts indicated in the following table.

TABLE 2

|                                                           | Fog  | Average Contrast | Relative Sensitivity | Maximum Density |
|-----------------------------------------------------------|------|------------------|----------------------|-----------------|
| Radio Type R                                              |      |                  |                      |                 |
| No addition                                               | 0.20 | 1.75             | 12.30                | 2.50            |
| Addition of Na <sub>2</sub> S <sub>2</sub> O <sub>3</sub> |      |                  |                      |                 |
| 0.10 g/liter                                              | 0.20 | 1.90             | 13.00                | 2.60            |
| 0.25 g/liter                                              | 0.20 | 2.10             | 13.80                | 2.77            |
| 0.50 g/liter                                              | 0.20 | 2.15             | 13.90                | 2.98            |
| 1.01 g/liter                                              | 0.20 | 1.75             | 13.80                | 3.00            |
| 2.02 g/liter                                              | 0.20 | 1.50             | 13.00                | 2.83            |
| Radio Type N                                              |      |                  |                      |                 |
| No addition                                               | 0.22 | 2.10             | 12.40                | 3.66            |
| Addition of Na <sub>2</sub> S <sub>2</sub> O <sub>3</sub> |      |                  |                      |                 |
| 0.25 g/liter                                              | 0.22 | 1.95             | 12.70                | 3.66            |
| 0.50 g/liter                                              | 0.23 | 2.05             | 13.20                | 3.69            |
| 1.01 g/liter                                              | 0.23 | 1.90             | 13.90                | 3.74            |
| 2.02 g/liter                                              | 0.24 | 1.80             | 14.40                | 3.74            |
| Radio Type Gamma                                          |      |                  |                      |                 |
| No addition                                               | 0.23 | 1.60             | 7.80                 | >4.00           |
| Addition of Na <sub>2</sub> S <sub>2</sub> O <sub>3</sub> |      |                  |                      |                 |
| 0.25 g/liter                                              | 0.23 | 1.90             | 8.85                 | >4.00           |
| 0.50 g/liter                                              | 0.24 | 1.80             | 9.00                 | >4.00           |
| 1.01 g/liter                                              | 0.30 | 1.95             | 10.20                | >4.00           |
| 2.02 g/liter                                              | 0.30 | 1.75             | 11.30                | >4.00           |
| Radio Type Lambda                                         |      |                  |                      |                 |
| No addition                                               | 0.29 | 2.45             | 8.00                 | >4.00           |
| Addition of Na <sub>2</sub> S <sub>2</sub> O <sub>3</sub> |      |                  |                      |                 |
| 0.25 g/liter                                              | 0.26 | 2.10             | 7.80                 | >4.00           |
| 0.50 g/liter                                              | 0.24 | 1.95             | 8.50                 | >4.00           |
| 1.01 g/liter                                              | 0.24 | 1.50             | 8.95                 | >4.00           |
| 2.02 g/liter                                              | 0.31 | 1.40             | 9.00                 | >4.00           |
| Radio Type Lambda                                         |      |                  |                      |                 |
| No addition                                               | 0.19 | 1.65             | 13.60                | 2.54            |
| Addition of KCNS                                          |      |                  |                      |                 |
| 0.10 g/liter                                              | 0.19 | 1.65             | 13.40                | 2.54            |
| 0.25 g/liter                                              | 0.19 | 1.70             | 13.25                | 2.54            |
| 0.50 g/liter                                              | 0.19 | 1.75             | 13.40                | 2.58            |
| 1.01 g/liter                                              | 0.20 | 1.75             | 13.50                | 2.64            |
| 2.02 g/liter                                              | 0.20 | 1.65             | 14.50                | 2.73            |
| Radio Type N                                              |      |                  |                      |                 |
| No addition                                               | 0.22 | 2.05             | 12.80                | 3.77            |
| Addition of KCNS                                          |      |                  |                      |                 |
| 0.25 g/liter                                              | 0.22 | 2.10             | 11.15                | 3.76            |
| 0.50 g/liter                                              | 0.23 | 2.10             | 13.40                | 3.78            |
| 1.01 g/liter                                              | 0.22 | 1.90             | 13.50                | 3.80            |

TABLE 2-Continued

|                          | Fog  | Average Contrast | Relative Sensitivity | Maximum Density |
|--------------------------|------|------------------|----------------------|-----------------|
| 2.02 g/liter             | 0.23 | 2.10             | 13.80                | 3.76            |
| <u>Radio Type Gamma</u>  |      |                  |                      |                 |
| No addition              | 0.22 | <1.50            | 10.00                | >4.00           |
| Addition of KCNS         |      |                  |                      |                 |
| 0.25 g/liter             | 0.23 | <1.50            | 9.70                 | >4.00           |
| 0.50 g/liter             | 0.24 | <1.50            | 9.90                 | >4.00           |
| 1.01 g/liter             | 0.26 | <1.50            | 11.20                | >4.00           |
| 2.02 g/liter             | 0.36 | <1.50            | 18.00                | >4.00           |
| <u>Radio Type Lambda</u> |      |                  |                      |                 |
| No addition              | 0.23 | 2.50             | 7.80                 | >4.00           |
| Addition of KCNS         |      |                  |                      |                 |
| 0.25 g/liter             | 0.24 | 2.70             | 7.80                 | >4.00           |
| 0.50 g/liter             | 0.26 | 2.90             | 8.25                 | >4.00           |
| 1.01 g/liter             | 0.28 | 2.80             | 8.25                 | >4.00           |
| 2.02 g/liter             | 0.28 | 2.50             | 8.75                 | >4.00           |
| <u>Radio Type R</u>      |      |                  |                      |                 |
| No addition              | 0.20 | 1.55             | 13.20                | 2.58            |
| Addition of Thio-urea    |      |                  |                      |                 |
| 0.25 g/liter             | 0.78 | <1.50            | 10.25                | 2.72            |
| <u>Radio Type N</u>      |      |                  |                      |                 |
| No addition              | 0.23 | 2.10             | 12.15                | 2.74            |
| Addition of Thio-urea    |      |                  |                      |                 |
| 0.25 g/liter             | 0.34 | 1.95             | 10.75                | 3.30            |
| <u>Radio Type Gamma</u>  |      |                  |                      |                 |
| No addition              | 0.22 | <1.50            | 9.75                 | >4.00           |
| Addition of Thio-Urea    |      |                  |                      |                 |
| 0.25 g/liter             | 2.84 | <1.50            | 6.20                 | >4.00           |
| <u>Radio Type Lambda</u> |      |                  |                      |                 |
| No addition              | 0.24 | <1.50            | 10.00                | 4.00            |
| Addition of Thio-urea    |      |                  |                      |                 |
| 0.25 g/liter             | 1.70 | 3.10             | 5.50                 | >4.00           |

## EXAMPLE 3

A material for medical radiography, of the type suitable for rapid machine development (Kodak Medical X-Ray Film RP X-OMAT Rapid Processing) was radiographically exposed, then divided into two parts. The first part was processed by machine in Kodak X-OMAT M6-RP X-Ray Processor in a processing cycle of 90 seconds employing the development bath Kodak RP Medical X-OMAT Developer-Replenisher Type MX810 of Eastman Koda. The second part was processed in a manual processing cycle comprising a development bath wholly analogous to solution C of Example 1 but containing, according to the present invention, 0.5050 g of sodium thiosulfate per liter of solution.

The results are indicated in the following table.

TABLE 3

|        | Fog  | Relative Sensitivity | Average Contrast | Maximum Density |
|--------|------|----------------------|------------------|-----------------|
| Part 1 | 0.21 | 6.8                  | 2.59             | 3.31            |
| Part 2 | 0.20 | 7.0                  | 2.72             | 3.22            |

What is claimed is:

1. A liquid photographic developer having a pH of from about 10 to about 11 and comprising about 10 to about 30 grams per liter of hydroquinone and from about 0.3 to about 0.9 grams per liter of phenidone, said developer further comprising a source of thiosulfate ions in an amount equivalent, in thiosulfate ion, to from about 0.1 to about 1.0 grams per liter of sodium thiosulfate.
2. The liquid photographic developer of claim 1 wherein said thiosulfate ion source is an alkali metal or ammonium thiosulfate.
- 15 3. The liquid photographic developer of claim 1 wherein said source of thiosulfate ions is sodium thiosulfate or ammonium thiosulfate.
4. The liquid photographic developer of claim 3 wherein said source of thiosulfate ions is present in an amount corresponding, in thiosulfate ion, to from about 0.3 to about 0.6 grams per liter.
- 25 5. The liquid photographic developer according to claim 1 wherein the pH of said developer is from about 10.2 to about 10.5.
- 30 6. A method for the manual development of a machine processable photographic film which comprises manually treating said film in a liquid photographic developer having a pH of from about 10.0 to about 11.0 and comprising from about 10 to about 30 grams per liter of hydroquinone, from about 0.3 to about 0.9 grams per liter of phenidone, and a source of thiosulfate ions in an amount equivalent, in thiosulfate ion, to sodium thiosulfate in an amount ranging from about 0.1 to about 1.0 grams per liter.
- 40 7. The method according to claim 6 wherein said liquid photographic developer contains ammonium thiosulfate or sodium thiosulfate as said source of thiosulfate ion.
- 45 8. The method according to claim 6 wherein said source of thiosulfate ions is present in an amount equivalent, in thiosulfate ion, to from about 0.3 to about 0.6 grams per liter of sodium thiosulfate.
- 50 9. The method according to claim 6 wherein the pH of said liquid photographic developer ranges from about 10.2 to about 10.5.
- 55 10. The method according to claim 6 wherein the photographic film is radiographic film.

\* \* \* \* \*